

## UNITED STATES PATENT OFFICE

2,339,267

## ELECTROLYTIC RECORDING

John V. L. Hogan, Forest Hills, Hugh C. Ressler,  
West Brighton, and William H. Tribble, Brooklyn, N. Y., assignors, by mesne assignments, to  
Faximile, Inc., New York, N. Y., a corporation of  
Delaware

No Drawing. Application April 15, 1940,  
Serial No. 329,828

1 Claim. (Cl. 204—2)

The present invention concerns materials for, and processes of electrolytic recording.

One object of the present invention is to provide methods of preparing recording carriers or sheets which will keep substantially unaltered for long periods prior to recording and which will yield records which will not fade or discolor for long periods after recording.

Another object is to increase the sharpness of recorded images by preventing fringes from forming during and after the instant of recording.

A further object is to provide an electrolytic recording material which is easily and cheaply prepared and which will yield superior recordings.

A still further object is to provide a process of and material for recording electrolytically which will produce a dense, sharp and permanent mark against a contrasting or white sheet at a high rate of linear recording speed.

These and other objects will be evident from the detailed description of the invention.

It is well known in the art of electrochemical recording that a mark may be obtained by the electrolytic deposition of a metal, such as silver, of a colored compound, such as lead peroxide, or of an adsorption complex, such as starch-iodine, on a paper support or other suitable carrier. It is less commonly known that as the speed of recording is increased, most of the materials which are satisfactory at low speed become useless.

While it may seem that it should be possible to compensate for the decrease in deposition time by a proportional increase in current, so that the work done is the same regardless of the elapsed time, practical considerations definitely limit the extent to which this compensating current increase may be utilized under any given conditions. Among the major limiting factors is current density, which must be kept well below the point at which thermal decomposition of the sensitizing ingredients, or of the carrier occurs. Another factor is electrode overvoltage, which does not necessarily increase at the same rate as does the current density, and hence the oxidation or reduction intensity that is required to produce a suitable change of color may not be reached until thermal decomposition is appreciable, and loss of detail and other undesirable effects result.

The materials and processes of the present invention are suitable for recording with an effective recording electrode area of 0.0001 square

inch moving with a linear speed of thirty inches a second or more.

It has been found that impregnation of the carrier just prior to marking has a number of disadvantages. It requires additional space at the recorder for the impregnating equipment. It requires attention to maintain liquid levels, etc. Most important, as far as the finished product is concerned, is the fact that impregnation of the support just prior to marking makes difficult the proper distribution and control of moisture in the record sheet at the point of marking.

The present invention concerns processes of impregnation in which the paper or other carrier is treated and processed to produce even distribution of moisture content which may be adjusted to any desired point. Thus, with sufficient time available, a paper which is much less porous and having a high wet strength may be used as the support. A much more even distribution of moisture may be obtained, yielding a more even record. The present invention contemplates using materials which will preserve the prepared support without discoloration over long periods of time prior to marking. It also contemplates storage of the prepared support in a humidor in order to maintain its moisture content within the optimum range until the time of recording. A suitable humidor is disclosed in Patent No. 2,111,776, entitled "Recording paper system," issued on March 22, 1938, to John V. L. Hogan.

It has been found, according to the present invention, that color-lakes may be used for high speed electrolytic recording on pretreated supports. Among the aromatic bodies which have been found suitable for use, according to the present invention, are those which have two or more adjacent hydroxy groups, and phenolic acids in which the carboxyl group may be part of the lake-forming configuration, such as the ortho hydroxy acids. It has been found that carriers impregnated with these lake-forming materials will keep without discoloration for long periods of time if sufficiently acid. Those which are not sufficiently acid in themselves may be kept by adding a source of hydrogen ions more highly ionized than the lake-forming compound, such as an acid which is stronger than the lake-forming material. The quantity of acid must be such that the impregnated support is maintained without discoloration prior to marking, but it must be insufficient to bleach the desired marks after recording. The electrolytes which are suitable for use in the present recording process are those which form strong bases under the action

of the recording current. The hydroxyl ions thus formed appear in the record support at the electrode opposite the marking electrode and diffuse thru the support, neutralizing the acid at the point of marking, thus permitting the color lake to form. Too much acid cannot be properly neutralized. A slight excess of acid may be taken care of by raising the recording current thereby generating more hydroxyl ions, but the sensitivity is thus reduced.

It has been found, according to the present invention, that the added acid has an important and unexpected result in that it greatly increases the sharpness and detail of the final record. To accomplish this result, the acid in the support must be present in sufficient amount to remove any fringes from the mark, but insufficient to damage the mark itself. This has been found to be possible, since the amount of lake formed in the fringes is very much less than that in the desired mark. Hence, while some of the mark may be bleached by the acid, enough remains to give to the eye of the observer the impression of completeness, whereas the fringe is apparently entirely removed. This leaves the colored deposit only in the area of maximum density, which is the area directly under the recording electrode at the instant of the passage of recording current. The fringe is apparently due to the ions which do not move directly thru the support upon the passage of current, and also to subsequent diffusion.

The amount of acid necessary to accomplish the above result will vary somewhat with the nature of the acid, the concentration of the electrolyte, and the marking current. The current in turn, is dependent upon the thickness and density of the paper, the moisture content, and the tinctorial power of the lake that is being formed. In general, 2 to 4 percent of the weight of the solid materials or 0.5 percent of the liquid, of acid of the strength of oxalic acid or an amount of other acids chemically equivalent to this may be used.

It has been found that when parchment type paper is used, a very thin sheet is suitable, because of its density and high wet-strength. A suitable grade is 0.0025 inch thick. For this type of paper, it has been found that a 20 percent solution of a uni-univalent electrolyte, such as sodium chloride, potassium chloride, sodium nitrate or potassium nitrate may be used with about 0.5 percent of an acid, such as oxalic or maleic for the purpose of preventing fringes. Any acid may be used as long as it is strong enough for the purpose and not so strong that it substantially weakens or discolors the support when in the quantity used.

The ingredients of the preferred impregnating material, according to the present invention, are: a lake-forming aromatic compound, an electrolytically conductive salt of a strong base, an acid more highly ionized than the lake-forming aromatic compound, and water in proper proportions.

As a particular example, a sheet of parchment paper is impregnated with the following materials:

|                    |                   |     |
|--------------------|-------------------|-----|
| Pyrocatechin       | grams             | 5   |
| Sodium nitrate     | do                | 5   |
| Potassium chloride | do                | 5   |
| Oxalic acid        | do                | 0.5 |
| Water              | cubic centimeters | 100 |

pass the sheet thru a bath made up of the above. The moisture is allowed to distribute itself evenly throughout the paper. This takes several hours in the case of parchment paper. The impregnated paper may be stored in a humidor until the time of recording. At the instant of recording, the impregnated support must contain sufficient moisture for the hydroxyl ions to migrate from the back of the support to the front, in order that the acid at the point of marking may be neutralized and the color-lake formed. The moisture must not be too great or diffusion of the mark will take place and loss of detail will result. Recording is accomplished by scanning the prepared paper with an electrode at least partly composed of a lake-forming metal and passing a modulated recording current thru the electrode and paper, in accordance with the subject matter to be recorded.

Another impregnating solution, according to the present invention, may be made by mixing the following:

|                                |                   |     |
|--------------------------------|-------------------|-----|
| Sodium catechol mono sulfonate | grams             | 8   |
| Sodium nitrate                 | do                | 15  |
| Maleic acid                    | do                | 0.4 |
| Water                          | cubic centimeters | 100 |

Still another impregnating formula is as follows:

|                             |                   |     |
|-----------------------------|-------------------|-----|
| Sodium naphthol disulfonate | grams             | 10  |
| 1:2:6                       | grams             | 10  |
| Potassium nitrate           | do                | 10  |
| Phosphoric acid             | do                | 0.5 |
| Water                       | cubic centimeters | 100 |

Lake-forming metals, according to the present invention, are those metals which, under the conditions of recording, form hydroxide or basic salts that are capable of entering into combination with the aromatic bodies in the impregnated support to form colored compounds called colored lakes, which normally are only slightly, if at all, soluble in water.

Among the preferred lake-forming metals suitable for the recording electrode are iron, chromium, copper, and nickel. It has been found that increased detail in the record may be obtained by alloying a hardening metal with the above lake-forming metals. One of the best alloys has been found to be stainless steel containing about 5 percent molybdenum. The molybdenum lakes are light colored and hence this metal may be used in the recording electrode to increase detail and decrease the rate of solution of the electrode without appreciably altering the color intensity of the final record.

According to the present invention, the impregnating material includes polyhydroxy phenols in which at least two hydroxyl groups are in the 1: 2 position, or a combination, such as an ortho amino phenol, or acetylated amino group, is converted during the electrolysis of recording to a hydroxy body which will form a lake. Substituted di hydroxy phenols, such as their sulfonic acids, amino compounds, chlor or brom derivatives, are also suitable, as are the mono and di carboxylic acids, and their homologues. In short, it has been found that substituent groups do not affect the lake-forming properties, provided the more acid substituents are converted in part, at least, to their salts, in order that this acidity be not so great that lake formation is hindered to an undesirable extent. Typical of the homologues are methyl di hydroxy benzene and naphthalene di-ol.

For the electrolytic conductors, we prefer univalent salts, because these have the highest ionic velocities for a given potential gradient and hence the highest conductivities. Thus, the chlorides, bromides, and nitrates of caesium, rubidium, potassium, sodium or lithium are to be preferred. Less desirable, but still usable, are salts which have reducing properties, such as sulfites and thiocyanates, since the recording process includes oxidation at the anode and with these salts some of the recording power goes to oxidize their ions.

We further prefer salts whose ions, both positive and negative, are easily confined to the area in which they are discharged, so as to limit lateral diffusion. The chloride and nitrate ions confine their attack upon the recording electrode to a very small area, whereas the sulfite ion tends to diffuse its attack. Similarly, ammonium salts are found to be very undesirable, because the ammonium ion, when discharged, forms gaseous  $\text{NH}_3$  which diffuses over a relatively wide area, forming ammonium hydroxide in locations that may be quite remote from the point of discharge. This diffusion causes fringes to form, and may leave insufficient  $\text{OH}$  ions at the desired marking point to neutralize the acid, so that the color lake cannot form properly.

It has been found, according to the present invention, that high speed recording requires sufficient lake-forming aromatic compound in the prepared support to yield a good mark. This requirement is met if the lake-forming aromatic compound has sufficient solubility in water. It has been found that a solubility of 3 percent or 30 greater in water at 25 degrees centigrade is sufficient.

The finished record keeps best when dry. The impregnated support may be allowed to dry naturally after recording or artificial means may be used, such as a heater or a draft of air. The 5 heat generated by the recording current may also be utilized to speed drying. In addition, the recording electrode may be heated by means of an auxiliary heating current, so that the record emerges from the recording point in a substantially dry condition.

While only a few examples have been given, according to the present invention, its many possible modifications will be evident to those skilled in the art within the spirit and scope of the invention, as set forth in the appended claim.

What is claimed is:

An electrolytic recording material, for recording by means of an electrode containing lake-forming metal, said recording material being carried by an inert support, said recording material consisting essentially of an aqueous solution of at least one non-volatile electrolyte chosen from the group consisting of chlorides, bromides and nitrates of caesium, rubidium, potassium, sodium or lithium for conducting an electric recording current, at least one lake-forming polyhydroxy phenolic compound for combining with the metal electrode to form a colored mark, and at least one acid chosen from the group consisting of oxalic and maleic in quantity of about two to four percent of the solid matter in said recording material for preserving the record, said composition being substantially free from lake-forming metals.

JOHN V. L. HOGAN.  
HUGH C. RESSLER.  
WILLIAM H. TRIBBLE.